

# UNITED STATES PATENT OFFICE.

CLAYTON L. BAKER AND MATHIAS THORKELSON, OF MOLINE, ILLINOIS.

## PAINT.

SPECIFICATION forming part of Letters Patent No. 423,656, dated March 18, 1890.

Application filed December 13, 1889. Serial No. 333,652. (No specimens.)

*To all whom it may concern:*

Be it known that we, CLAYTON L. BAKER and MATHIAS THORKELSON, of Moline, Illinois, have invented a certain new and useful Improvement in Paint, of which the following is a specification.

Our improved paint is particularly adapted for priming or first coat of wood and iron work; and it consists of the following ingredients, compounded in the manner and about the proportions stated, that is to say: We take of raw linseed-oil, thirty-six parts; lamp-black, nine parts; coach-japan, eleven parts; turpentine, twenty-two parts; iron-ore or mineral paint, one hundred parts; and after thoroughly mixing said ingredients we allow the mass to stand for a time—say twelve hours—and then grind in an ordinary paint-mill.

The iron-ore or mineral paint is a natural product, which is well known and which contains, usually, silica, alumina, lime, and other ingredients in varying proportions.

The proportions above stated may be varied within certain limits; but those here given have been found to be the best for the work named.

This paint is found to adhere well because of the fact that it readily penetrates wood, gives a uniform body and surface, and can be readily and conveniently applied by a common brush by an unskilled laborer, and can be smoothed by sand-paper or in other ways without injury or without rubbing off.

We claim—

The herein-described paint, composed of raw linseed-oil, lamp-black, coach-japan, turpentine, and natural-mineral paint, in about the proportions stated, substantially as described.

CLAYTON L. BAKER.

MATHIAS THORKELSON.

Witnesses:

ELMER E. MORGAN,  
W. E. KRATZER.